

May 6, 1941.

C. F. ALBAN ET AL

2,240,824

ELECTRICAL RESISTOR OF THERMOFLEX MATERIAL

Filed Dec. 6, 1937

2 Sheets-Sheet 1



Fig. 1



Fig. 2



Fig. 3



Fig. 4

INVENTORS  
Clarence F. Alban  
Stanley R. Hood  
Barnes, Russell, Daughlin & Keim  
ATTORNEYS

BY

May 6, 1941.

C. F. ALBAN ET AL

2,240,824

ELECTRICAL RESISTOR OF THERMOFLEX MATERIAL

Filed Dec. 6, 1937

2 Sheets-Sheet 2



INVENTORS  
Clarence F. Alban  
Stanley R. Hood  
Barnes, Kinselle, Daughlin & Reich  
ATTORNEYS

## UNITED STATES PATENT OFFICE

2,240,824

## ELECTRICAL RESISTOR OF THERMOFLEX MATERIAL

Clarence F. Alban and Stanley R. Hood, Detroit,  
Mich., assignors to W. M. Chace Company,  
Detroit, Mich., a corporation of Michigan

Application December 6, 1937, Serial No. 178,324

8 Claims. (Cl. 297—15)

This invention relates to an electrical resistor of thermoflex material.

As herein used the term "thermoflex material" denotes any composite material consisting of two or more laminae of metals or metal alloys, one lamina of which has a different coefficient of expansion than the other so that upon a change of temperature the metal will bend or flex due to the differential expansion of the said laminae. These thermoflex metals are commonly called thermostatic bimetal, thermostatic trimetal, and so on up the line depending upon how many laminae there are.

The known metal alloys suitable for use in thermoflex metal are limited in number and the physical and chemical laws governing their behavior are known. For example, to obtain the best presently available thermoflex materials or thermostatic bimetals having highest coefficient of deflection, it is customary with materials having approximately equal moduli of elasticity to make the high expanding lamina and low expanding lamina of approximately equal thickness. We have discovered that this physical law applies when more than two laminae are used to fabricate a given thermoflex material. In this invention it is necessary to classify the alloys or metals used into high or low expanding components as the situation may require. After this classification has been made, we have found it good practice to make the sum of the thicknesses of the low and high expanding laminae approximately equal.

We have also discovered that in the flow of electrical current through thermoflex metal that the laminae form a parallel circuit rather than a series circuit. This being true, the reciprocal of the equivalent resistance of the parallel circuit formed by thermoflex metal is the sum of the reciprocals of the individual resistances of the several laminae.

The use of thermoflex material as a resistor in an electrical circuit is not new. For example, circuit interrupters as well as circuit breakers of bimetallic thermoflex material are known. However, the application of thermoflex material as a resistor in an electrical circuit has been handicapped because the known metal alloys suitable for use in thermoflex material are limited in number. Since the known metal alloys suitable for use in thermoflex material are limited in number, the use of these thermoflex materials as electrical resistors is dependent upon the electrical resistivity of any standard length and section (for example, circular mil

foot) of these materials. The known metal alloys suitable for use in thermoflex material have very different resistivities measured in ohms per circular mil foot at a given temperature. By variation of analysis of these alloys, the resistivity of a standard length and section of thermoflex material can be varied within limits, but this impairs the deflectivity of the material.

Bimetal can be made having the low expanding lamina of invar (36% nickel, 64% iron) and the high expanding lamina of pure nickel. The difficulty with this bimetal is that its coefficient of deflection is much less than the best known alloys suitable for use in bimetal such for example, as an alloy for the low expanding lamina consisting of invar (36% nickel, 64% iron) and the high expanding side consisting of 22% nickel, 4 1/4% chromium and the remainder substantially iron. It will be noted that this second mentioned thermoflex material is the same as the one above-mentioned except that the high expanding lamina has a different composition. The difference in electrical resistivity per circular mil foot of these two bimetals is roughly four hundred ohms, but even by variation of analysis it has been found that at most only a few alloys suitable for use in thermoflex material can be obtained. The bimetals made from these few alloys have different resistivities per circular mil foot, but when arranged in order from the lowest to the highest resistivity per circular mil foot, it is found that there is a considerable hiatus between the resistivities of most thermoflex materials. Therefore it is impossible, using a standard length and section of thermoflex material, to fabricate a set of resistors having resistivities covering a desired range. For example, if it were required to fabricate a set of thermoflex elements for use in electrical circuits having amperage ratings of 10, 15, 20, 25, 30, 35, 40, 45, and 50, it would have been heretofore impossible because of the above-mentioned facts pertaining to thermoflex material. Therefore, it is the object of this invention to overcome the above-mentioned limitation in the use of thermoflex material as an electrical resistor and to produce a thermoflex material which will permit the fabrication of electrical resistors having any desired resistivity or amperage rating per given standard length and standard cross section.

Three constant conditions must be taken into consideration whenever thermoflex material is being made to be used as a resistor in an electrical circuit: namely, (1) the low expansion

lamina of the thermoflex material should approximate one-half the total thickness of the thermoflex material; (2) the compositions of alloys suitable for laminae in thermoflex material are fairly well fixed and limited; (3) the thermoflex material conducts currents as a parallel circuit.

This object has been achieved by incorporating in our new thermoflex material, either as an intermediate or outer lamina or laminae, a lamina or laminae of a metal or metal alloy having high electrical conductivity. Among these metals may be mentioned nickel, copper, cobalt, silver, gold, aluminum, platinum, manganese, iron, chromium, molybdenum, tungsten and alloys containing these or other metals having a high electrical conductivity. As set forth in *Handbook of Chemistry and Physics*, 19th Ed. by Charles D. Hodgman, edition of September 1934, pages 1337 through 1343, the resistivity of each of the above metals measured in ohms per cubic centimeter at a temperature of 20° C. is as follows:

|                  |                       |
|------------------|-----------------------|
| Nickel -----     | $7.8 \times 10^{-6}$  |
| Copper -----     | $1.69 \times 10^{-6}$ |
| Cobalt -----     | $9.7 \times 10^{-6}$  |
| Silver -----     | $1.63 \times 10^{-6}$ |
| Gold -----       | $2.44 \times 10^{-6}$ |
| Aluminum -----   | $2.83 \times 10^{-6}$ |
| Platinum -----   | $10. \times 10^{-6}$  |
| Manganese -----  | $5. \times 10^{-6}$   |
| Iron -----       | $10. \times 10^{-6}$  |
| Chromium -----   | $2.6 \times 10^{-6}$  |
| Molybdenum ----- | $5.7 \times 10^{-6}$  |
| Tungsten -----   | $5.6 \times 10^{-6}$  |

All of the above metals have a high electrical conductivity within the meaning of the term as herein used, that is, a low electrical resistivity. Hence, as used herein the phrase "metal or metal alloy having high electrical conductivity" means any metal or metal alloy having an electrical resistivity measured as above and equivalent to the electrical resistivity of any of the above listed metals. According to the above-mentioned *Handbook of Chemistry and Physics*, the electrical resistivity measured as above of the following nickel steel alloys is as follows:

|                              |                     |
|------------------------------|---------------------|
| Invar (35% nickel) -----     | $81 \times 10^{-6}$ |
| 10% nickel, .1% cobalt ----- | $29 \times 10^{-6}$ |
| 25% nickel, .1% cobalt ----- | $39 \times 10^{-6}$ |

These alloys for the purposes of this description are considered as having a low electrical conductivity. Although no hard and fast line of division can be drawn between high and low electrical conductivity, the above-mentioned metals are considered as having high electrical conductivity whereas the above-mentioned nickel-steel alloys are considered as having a low electrical conductivity. Preferably these metals should be pure or have but a very small or inconsequential amount of impurities therein. This lamina of high conducting metal functions primarily as an electrical conductor and the other laminae function primarily to cause the flexing of the material incident to temperature change.

Since the resistivity of each of these pure metals is very easily computed and the resistance for any given length varies inversely with the cross sectional area of this pure metal lamina, and having discovered that the thermoflex material conducts current as a parallel circuit, the resistivity of the thermoflex material is varied by varying the thickness of the pure or high

conducting metal lamina. Further, since the low expanding lamina or component of the thermoflex metal must always at least approximate one-half of the sum of the thicknesses of all of the laminae, therefore the sum of the thicknesses of the high expanding lamina and the high conducting metal lamina is computed to approximately equal the thickness of the low expanding side. By increasing the thickness of the high conducting metal lamina relative to the thicknesses of the other laminae the resistance of the material per circular mil foot is decreased and by decreasing the thickness of the high conducting metal lamina the resistance of the thermoflex element per circular mil foot is increased.

By way of description rather than limitation there will now be described a method for fabricating an electrical resistor such as a circuit breaker element having any given resistivity. When it is proposed to use thermoflex material as a circuit breaker element, particularly for circuit breakers having a low amperage rating, say from 10 to 100 amperes, such as are suitable for domestic use, or having an amperage rating still lower such as are suitable for use in the electrical circuit of an automotive vehicle, then there must be taken into consideration a fourth constant condition, that is, that these breaker elements are manufactured in standard sizes. Hence, a breaker element having any given amperage rating, say 10 amperes, has to be made the same size as a circuit breaker element having another given amperage rating either more, such as 100 amperes, or less, say 1 ampere.

In the drawings:

Fig. 1 is a sectional view through a circuit breaker having a tripping or breaker element of thermoflex material showing the position of the elements when the circuit is completed and the current is flowing through the circuit.

Fig. 2 is a view similar to Fig. 1 showing the circuit breaker in tripped position and the circuit broken.

Fig. 3 and 4 show circuit breaker elements of standard size but having different resistivities.

Figs. 5, 6, 7 and 8 show electrical resistors of thermoflex material each showing the several different laminae arranged in different positions one relative to the other.

Referring to Fig. 1 the circuit breaker comprises a stationary electrically conducting contact 1, a contact bar 2 pivoted as at 3 upon the plunger 4, and a handle 5 pivoted as at 6 upon the case 7 which encloses the circuit breaker mechanism. A compression spring 8 is seated in a socket 9 in the base of the case 7 and engages the contact bar as at 10 to provide direct pressure upon the stationary contact 1 and the movable contact 11 carried by the contact bar 2. The spring 8 also acts through the contact bar 2 to provide a minor pressure upon the thermoflex element 20.

The contact bar is also connected to the thermoflex element 20 by a flexible lead 41 which is welded at each end to the thermoflex element 20 and contact bar 2.

The tripping or breaker element 20 is fabricated to have a predetermined amperage rating and is fixed at one end as at 22 to the mounting bracket 43. When the circuit breaker is in "on" position, as shown in Fig. 1, and current at or below the amperage rating of the tripping or breaking element 20 is flowing through the cir-

cuit, then contacts 1 and 11 are engaged. The current at this time is flowing through contacts 1, 11, contact bar 2, lead 41, thermoflex element 20 and bracket 23. Whenever the current flowing through this circuit is stepped up, e. g., when the circuit is shorted or overloaded, the temperature of the thermoflex tripping or breaker element 20 increases, when the overload reaches about 50% of the rated amperage, depending, of course, on the time, then the rise in temperature causes the thermoflex tripping element 20 to flex as indicated in Fig. 2. This releases the contact bar 2 and permits the spring 8 to pivot the contact bar 2 to the position shown in Fig. 2, thus disengaging or rupturing contacts 1 and 11. This breaks the circuit between contacts 1 and 11 and current ceases to flow through the circuit. At this time the handle 5 is shifted from the "on" position shown in Fig. 1 to "off" or tripped position shown in Fig. 2. When the cause of the short circuit or overload has been removed the circuit breaker may be reset by returning the handle 5 to "on" position. If the overload or short circuit remains in the circuit, then upon moving the handle to "on" position to again reset the circuit breaker, it will again overload the thermoflex tripping element 20 and cause the circuit breaker to trip as above described.

In Fig. 3 there is shown a circuit breaker element of standard size. This element 20 consists of a low expansion lamina 12, high expansion lamina 13 and an intermediate lamina 14 of high conductivity. When the lamina 12 is an alloy of 30% nickel, 8% cobalt and 62% iron having a thickness of .530 inch and the high conductivity lamina 14 has a thickness of .265 inch and consists of approximately pure nickel and the high expanding lamina 13 is an alloy consisting of 22% nickel, 4 1/4% chromium and the remainder substantially iron and a thickness of .265 inch, then the resistivity of this trimetal element is 150 ohms per circular mil foot at 80° F. This element has a high coefficient of deflection. It is not commercially practical to obtain 100% pure metal. Therefore the high conducting lamina 14 is preferably made from any of the above-mentioned high conducting metals but with a predetermined small amount of impurities therein such that the electrical resistivity can be controlled. Thus by the addition of small amounts of impurities to obtain the predetermined allowable amount of impurities a high conducting lamina 14 of the same resistivity can always be obtained.

To produce a circuit breaker element having a resistivity of 200 ohms per circular mil foot at 80° F., then, for the reason above defined, lamina 12 will have the same thickness of .530 inch but lamina 14 is decreased to .100 inch and the thickness of lamina 13 is increased to .430 inch.

To obtain higher resistivity per circular mil foot then it is proposed to use a thermoflex metal breaker element as shown in Fig. 4 in which the low expanding lamina 15 consists of 36% nickel and 64% iron and the high conducting lamina 16 consists of substantially pure nickel and the high expanding lamina 17 consists of 22% nickel and 4 1/4% chromium and the remainder substantially iron. To obtain a resistivity of 300 ohms per circular mil foot at 80° F., the thickness of lamina 15 is .530 inch; that of lamina 16, .085 inch; and lamina 17, .445 inch. To obtain a resistivity of this thermoflex metal of 350 ohms

per circular mil foot at 80° F., then lamina 15 remains the same thickness but lamina 16 is reduced to .055 inch and lamina 17 is increased in thickness to .475 inch. To obtain a resistivity of 400 ohms per circular mil foot at 80° F., the thickness of lamina 16 is decreased to .032 inch and the thickness of lamina 17 is increased to .498 inch. After the composite welded ingots are prepared as described by the foregoing examples, they are rolled by standard procedure to required thickness.

From the above it will be noted that the thickness of the low expanding lamina is .530 inch which is equal to the sum of the thicknesses of the other two laminae. In fabricating breaker elements of a standard size the thermoflex metal having the higher resistivity per circular mil foot is used for those breaker elements having a lower amperage rating, and the thermoflex metal having the lower resistivities are used for breaker elements having a higher amperage rating.

From the above it is evident that by gradually decreasing the thickness of the high conducting lamina 14 and correspondingly increasing the thickness of the high expanding lamina that one can obtain a thermoflex material having any resistivity desired within predetermined limits, for descriptive purposes shown as a trimetal, and having a high flexibility corresponding very favorably with the flexibility of the best thermoflex metals now known and produced. Thus, within a given range of amperage ratings there can be obtained for a standard size electrical resistor a set of resistors having increased amperage ratings in whatever progression desired.

In the resistor shown in Fig. 5 the two outer laminae 120 consist of a high conducting metal which can have a high coefficient of expansion such as nickel or a high electrical conducting metal having a low coefficient of expansion such as chromium, molybdenum or tungsten. Of the two intermediate laminae 121 and 122, 121 has a higher coefficient of expansion than 122. In such case lamina 121 can be made of a nickel-steel alloy containing 22% nickel and 4 1/4% chromium, and lamina 122 can consist of invar. For purposes of description, this type could be fabricated from a standard type of thermoflex, it only being necessary to plate or weld on high electrical conducting layers as laminae 120. It is, of course, understood that laminae 120 are not necessarily of similar materials or of exactly equal thickness. Thus, laminae 120, under most conditions, would be very thin and have little effect on the deflection properties of the thermoflex.

In the electrical resistor shown in Fig. 6 the lamina 23 has a high coefficient of expansion and can consist of a nickel-steel alloy comprising 22% nickel, 4 1/4% chromium. Lamina 24 can consist of a high electrical conducting metal or metal alloy having a low coefficient of expansion such as chromium, molybdenum or tungsten. The low coefficient lamina 25 can be invar. Here again the total thickness of laminae 24 and 25 equals that of lamina 23, that is, A equals B.

In Fig. 7 the lamina 26 has a low coefficient of expansion and can consist of invar whereas the lamina 27 has a high coefficient of expansion and can consist of the nickel-steel alloy having 22% nickel and 4 1/4% chromium. The two high conducting laminae 28 and 29 are positioned intermediate the laminae 26 and 27. The lamina 28 has a high electrical conductivity but a low

coefficient of expansion and can be made from chromium, molybdenum or tungsten. The lamina 29 has a high electrical conductivity and a high coefficient of expansion and can be made from nickel or copper, for example. Here again the total thickness of the laminae 26 and 28 equals that of 27 and 29, that is, A equals B. In Fig. 8 the electrical resistor has outer laminae 30 and 31 each having the same thickness, A equals B. Lamina 30 can be invar and the lamina 31 a nickel-steel alloy containing 22% nickel, 4 1/4% chromium which has a high coefficient of expansion. The intermediate lamina 32 has a high electrical conductivity and can be made from a metal such as nickel or copper having a high coefficient of expansion or from a metal such as chromium, molybdenum or tungsten having a low coefficient of expansion. In this form preferably the lamina 32 should be as thin as possible commensurate with the desired conductivity of the resistor because maximum deflectivity is obtained when the total thickness of the high expanding lamina or laminae will approximately equal the total thickness of the low expanding lamina or laminae.

The terms "high coefficient of expansion" and "low coefficient of expansion" are herein used in their relative sense. As is well-known in order to obtain any deflectivity in thermoflex material the one lamina must have a lower coefficient of expansion than the other. A given metal alloy or metal may be used as the high expanding lamina in one thermoflex material and the same given metal alloy or metal may be used as the low expanding lamina in another thermoflex material. In the first case the lamina will be referred to as the "high expanding lamina" whereas in the second case this lamina from the same metal or metal alloy will be referred to as the "low expanding lamina."

We claim:

1. An electrical resistor of thermoflex material having a high temperature coefficient of deflection, a predetermined cross section and length and electrical resistance consisting of a plurality of joined metallic laminae including a metallic lamina having a high thermal coefficient of expansion, a metallic lamina having a low thermal coefficient of expansion and at least one metallic lamina having a high electrical conductivity and a cross sectional area correlated with respect to the cross sectional areas and electrical resistances of said above mentioned laminae to obtain said predetermined resistance whereby the deflection rate is maintained substantially the same throughout a wide range of cross sectional areas for said high conducting lamina.

2. An electrical resistor of thermoflex material having a high temperature coefficient of deflection, a predetermined cross section and length and electrical resistance consisting of a plurality of joined metallic laminae including a metallic lamina having a high thermal coefficient of expansion, a metallic lamina having a low thermal coefficient of expansion and at least one metallic lamina having a high electrical conductivity, and a cross sectional area correlated with respect to the cross sectional areas and electrical resistances of said above mentioned laminae to obtain said predetermined resistance whereby the deflection rate is maintained substantially the same throughout a wide range of cross sectional areas for said high conducting lamina, the thickness of the metallic

lamina having a low thermal coefficient of expansion being approximately equal to the sum of the thicknesses of the lamina having a high coefficient of expansion and the lamina having a high electrical conductivity.

3. An electrical resistor of thermoflex material having a high temperature coefficient of deflection, a predetermined cross section and length and electrical resistance consisting of a plurality of joined laminae including a lamina of an alloy having a high thermal coefficient of expansion from the group of alloys consisting of iron-nickel alloy, iron-nickel-chromium alloy, and iron-nickel-manganese alloy, a lamina of a nickel-iron alloy having a higher nickel content than the above-mentioned laminae and a low thermal coefficient of expansion and a metallic lamina having a high electrical conductivity and a cross sectional area correlated with respect to the cross sectional areas and electrical resistances of said above mentioned laminae to obtain said predetermined resistance whereby the deflection rate is maintained substantially the same throughout a wide range of cross sectional areas for said high conducting lamina.

4. An electrical resistor of thermoflex material, a predetermined cross section and length and electrical resistance consisting of a plurality of joined laminae including a lamina of an alloy having a high thermal coefficient of expansion from the group of alloys consisting of iron-nickel alloy, iron-nickel-chromium alloy, and iron-nickel-manganese alloy, a lamina comprising a nickel-iron alloy having a low thermal coefficient of expansion, and an intermediate metallic lamina having a high electrical conductivity and a cross sectional area correlated with respect to the cross sectional areas and electrical resistances of said above mentioned laminae to obtain said predetermined resistance whereby the deflection rate is maintained substantially the same throughout a wide range of cross sectional areas for said high conducting lamina, the ratio of the nickel to the iron content in each of the first two mentioned laminae being such that the thermoflex material has a high flexivity.

5. An electrical resistor of thermoflex material having a high temperature coefficient of deflection, a predetermined cross section and length and electrical resistance consisting of a plurality of joined metallic laminae including a metallic lamina having a high thermal coefficient of expansion and a low electrical conductivity, a metallic lamina having a low thermal coefficient of expansion and a low electrical conductivity and at least one metallic lamina positioned between the above-mentioned laminae having a high electrical conductivity and a coefficient of expansion intermediate to that of one of the above laminae and a cross sectional area correlated with respect to the cross sectional areas and electrical resistances of said above mentioned laminae to obtain said predetermined resistance whereby the deflection rate is maintained substantially the same throughout a wide range of cross sectional areas for said high conducting lamina, the total thickness of the high expanding lamina or laminae being approximately equal to that of the low expanding lamina or laminae.

6. An electrical resistor of thermoflex material having a high temperature coefficient of deflection, a predetermined cross section and length and electrical resistance consisting of a plurality of joined metallic laminae including a

metallic lamina having a high thermal coefficient of expansion, a metallic lamina having a low thermal coefficient of expansion and at least one lamina of nickel having a high electrical conductivity and a cross sectional area correlated with respect to the cross sectional areas and electrical resistances of said above mentioned laminae to obtain said predetermined resistance whereby the deflection rate is maintained substantially the same throughout a wide range of cross sectional areas for said high conducting lamina.

7. An electrical resistor of thermoflex material having a high temperature coefficient of deflection, a predetermined cross section and length and electrical resistance consisting of a plurality of joined metallic laminae including a metallic lamina having a high thermal coefficient of expansion, a metallic lamina having a low thermal coefficient of expansion and at least one lamina of copper having a high electrical conductivity and a cross sectional area correlated with respect to the cross sectional areas and electrical resistances of said above mentioned laminae to

obtain said predetermined resistance whereby the deflection rate is maintained substantially the same throughout a wide range of cross sectional areas for said high conducting lamina.

- 5 8. An electrical resistor of thermoflex material having a high temperature coefficient of deflection, a predetermined cross section and length and electrical resistance consisting of a plurality of joined metallic laminae including a metallic lamina having a high thermal coefficient of expansion, a metallic lamina having a low thermal coefficient of expansion and at least one lamina of iron having a high electrical conductivity and a cross sectional area correlated with respect to the cross sectional areas and electrical resistances of said above mentioned laminae to obtain said predetermined resistance whereby the deflection rate is maintained substantially the same throughout a wide range of cross sectional areas for said high conducting lamina.
- 10 15 20

CLARENCE F. ALBAN.  
STANLEY R. HOOD.